

1

3,389,205

## METHOD OF IMPROVING THE DYE RECEP- TIVITY OF FIBERS OF VINYLIDENE CY- ANIDE COPOLYMERS

Saunders E. Jamison, Summit, and William J. Roberts, Bernardsville, N.J., assignors to Celanese Corporation, a corporation of Delaware  
No Drawing. Filed Mar. 24, 1964, Ser. No. 354,452  
19 Claims. (Cl. 264—178)

### ABSTRACT OF THE DISCLOSURE

A method for producing vinylidene cyanide copolymer fibers of superior dye receptivity wherein the fibers are produced by extruding a spinning solution of vinylidene cyanide copolymer into a coagulation bath containing a minor amount of a polyoxyalkylene glycol and/or fatty acid esters of polyoxyalkylene glycols. The vinylidene cyanide copolymer spinning solution preferably utilizes a solvent comprised of a major proportion of acetonitrile in a minor proportion of water and the coagulation bath preferably utilizes a major proportion of water and a minor proportion of acetonitrile in addition to the minor proportion of polyoxyalkylene material.

This invention relates to synthetic fibers exhibiting improved dye receptivity and to a method of preparing the same. More particularly, this invention relates to vinylidene cyanide copolymer fibers having superior dye receptivity, such fibers having been prepared by extruding a spinning solution containing vinylidene cyanide copolymer into a coagulating bath containing a minor amount of a material selected from the group consisting of polyoxyalkylene glycols and fatty acid esters of polyoxyalkylene glycols, to thereby wet-spin fibers from such spinning solutions.

Synthetic resinous copolymers of vinylidene cyanide and another monomer copolymerizable therewith are known to present valuable fiber-forming characteristics. However, heretofore the resulting fibers have been difficult to dye satisfactorily, e.g., the percent dye uptake by the fibers has been undesirably low.

The resinous copolymers of vinylidene cyanide which are contemplated herein generally contain in excess of about 45% of vinylidene cyanide (methylene malononitrile or vinylidene dinitrile) units copolymerized with one or more ethylenically unsaturated monomers such as vinyl acetate or the like, as described in U.S. Patents 2,615,865 through 2,615,880, inclusive, 2,628,954, 2,650,911, 2,654,724, 2,654,728, 2,657,197, 2,716,104, 2,716,105, 2,716,106, and 2,740,769 and Canadian Patent No. 569,262.

The copolymers usually comprise units of vinylidene cyanide alternated with one or more copolymerizable monomers selected from the following classes of compounds;

(1) Vinyl esters of aliphatic monocarboxylic acids, preferably of the structure  $RCOOH$ , wherein R is an alkyl, such as vinyl acetate, vinyl propionate, vinyl butyrate, vinyl isobutyrate, vinyl valerate, vinyl caproate, vinyl enanthate and the like. The copolymerization with vinylidene cyanide of such copolymerizable monomers and the resulting copolymers are described more fully in U.S. Patent 2,615,866, issued Oct. 28, 1952.

(2) Vinyl esters of the structure



2

wherein Ar is an aromatic radical in which all the hydrogen atoms are attached to carbon atoms, such as vinyl benzoate; homologs of vinyl benzoate of the formula



10 wherein each R is a member of the class consisting of hydrogen atoms or lower alkyl radicals, for example, vinyl toluate and the like; monomers of the above general class wherein the aromatic radical is halogen substituted, such as vinyl p-chlorobenzoate, vinyl o-chlorobenzoate, vinyl m-chlorobenzoate, and similar vinyl halobenzoates and monomers of the above general class wherein the aromatic radical is alkoxy substituted, for example, vinyl p-methoxybenzoate, vinyl o-methoxybenzoate and vinyl p-ethoxybenzoate. The copolymerization with vinylidene cyanide, of such monomers, and the resulting copolymers are disclosed in U.S. Patent 2,615,867, issued Oct. 28, 1952.

(3) Styrene and substituted styrenes of the general formula



30 wherein Ar is an aromatic radical in which all of the hydrogen atoms are attached to carbon atoms and R is a member of the class consisting of hydrogen atoms and alkyl radicals, preferably those which contain from 1 to 4 carbon atoms, such as styrene itself, and substituted styrenes such as alpha-methyl styrene, alpha-ethyl styrene, alpha-butyl styrene, alpha-chlorostyrene, alpha-bromostyrene, 2,5-dichlorostyrene, 2,5-dibromostyrene, ortho-, meta-, and paramethoxystyrene, paraalpha-dimethyl styrene, paramethyl styrene, 3,4-dichlorostyrene, 3,4-difluorostyrene, 2,4-dichlorostyrene, 2,4,5-trichlorostyrene, dichloromonofluorostyrenes and the like. Copolymerization of vinylidene cyanide with styrene and substituted styrenes is disclosed in U.S. Patent 2,615,868, issued Oct. 28, 1952;

(4) Olefins of the general structure



50 wherein R is an alkyl radical, preferably containing from 1 to 6 carbon atoms, such as isobutylene, 2-methyl propene-1, 2-methyl-butene-1, 2-methylpentene-1, 2,3-dimethylbutene-1, 2,3-dimethyl-pentene-1, 2,3,3-trimethylbutene-1, 2,3,4-trimethylpentene-1, 2,6-dimethyloctene-1, 2-methylnonadecene-1, and the like. Copolymerization of such olefins with vinylidene cyanide is disclosed in U.S. Patent 2,615,865, issued Oct. 28, 1952;

(5) Alkyl esters of methacrylic acid which possess the structure



60 65 70 wherein R is an alkyl radical, preferably containing from 1 to 8 carbon atoms, for example, methyl methacrylate, ethyl methacrylate, propyl methacrylate, butyl methacrylate, amyl methacrylate, hexyl methacrylate, heptyl methacrylate, octyl methacrylate, decyl methacrylate, and the like. Vinylidene cyanide/alkyl methacrylate copolymers and their preparation are disclosed in U.S. Patent 2,615,871, issued Oct. 28, 1952;

(6) 2-halogenated monoolefins of the structure



wherein R is a lower alkyl radical such as methyl, ethyl, propyl or butyl, and Y is a halogen atom, such as 2-chloropropene, 2-chlorobutene, 2-chloropentene, 2-chlorohexene, 2-chloroheptene, 2-bromobutene, 2-bromoheptene, 2-fluorohexene, 2-fluorobutene, 2-iodopropene, 2-iodopentene, and the like. Copolymerization of these compounds with vinylidene cyanide is disclosed in U.S. Patent 2,615,877, issued October 28, 1952;

(7) Isopropenyl esters of organic monocarboxylic acids, preferably of the formula RCOOH, wherein R is an alkyl radical containing from 1 to 6 carbon atoms, and including isopropenyl acetate, isopropenyl propionate, isopropenyl isobutyrate, isopropenyl valerate, isopropenyl caproate, and isopropenyl enanthate; as well as isopropenyl esters of aromatic carboxylic acids, for example, isopropenyl benzoate, isopropenyl p-chlorobenzoate, isopropenyl o-chlorobenzoate, isopropenyl m-chlorobenzoate, isopropenyl toluate, isopropenyl alpha-chloroacetate, isopropenyl alpha-bromopropionate, and the like; the copolymerization of all of which with vinylidene cyanide is described in U.S. Patent 2,615,875, issued Oct. 28, 1952;

(8) Vinyl esters of alpha-halo saturated aliphatic monocarboxylic acids of the structure



wherein R is a member of the class consisting of hydrogen and an alkyl radical, preferably a lower alkyl radical, and Y is a halogen atom, such as vinyl alpha-chloroacetate, vinyl alpha-bromoacetate, vinyl alpha-iodopropionate, vinyl alpha-bromovalerate and the like. The copolymerization of such monomers with vinylidene cyanide is described in U.S. Patent 2,615,876, issued Oct. 28, 1952.

(9) Vinyl halides such as vinyl chloride, vinyl bromide and the like, which are copolymerized with vinylidene cyanide as described in U.S. Patent 2,615,869, issued Oct. 28, 1952.

In addition to interpolymers of vinylidene cyanide containing the essentially 1 to 1 molar alternating structure and essentially 50 mol percent vinylidene cyanide units, such as those disclosed in the patents referred to above, other vinylidene cyanide interpolymers have been described. For example, there are included interpolymers, of this vinylidene cyanide content, made from vinylidene cyanide and more than one copolymerizable monoolefinic compound, at least one of which forms an essentially 1:1 alternating copolymer when copolymerized with vinylidene cyanide, a large number of which interpolymers are disclosed in U.S. Patent 2,716,106.

Other polymerizable monoolefinic compounds form interpolymers with vinylidene cyanide, in addition to those set out above including, by way of example, the following classes of compounds:

Monoolefinic hydrocarbons, such as 2,3-dimethylhexene-1; 2,3,4-trimethyl-pentene-1; ethylene; propylene; butylene; amylene; hexylene and the like;

Esters of unsaturated acids other than methacrylic, e.g., of acrylic acid and tiglic acid such as methyl acrylate, ethyl acrylate, propyl acrylate, isopropyl acrylate, amyl acrylate, 3,5,5-trimethylhexyl acrylate, dodecyl acrylate and ethyl tiglate.

Allyl and substituted allyl esters such as allyl chloride, allyl cyanide, allyl bromide, allyl fluoride, allyl iodide, allyl nitrate, allyl thiocyanate, allyl butyrate, allyl benzoate, allyl 3,5,5-trimethyl hexoate, allyl lactate, allyl pyruvate, allyl acetoacetate, allyl thioacetate, as well as methallyl esters corresponding to the above allyl esters as well as esters from such alkenyl alcohols as betaethyl allyl alcohol, beta-propyl allyl alcohol, and 1-butene-4-ol;

Esters of substituted acrylic acids, such as methyl alpha-chloroacrylate, methyl alpha-bromoacrylate, ethyl alpha-chloroacrylate, propyl alpha-chloroacrylate, amyl alpha-chloroacrylate, 3,5,5-trimethyl hexyl alpha-chloroacrylate and decyl alpha-cyanoacrylate;

Esters of monoethylenically unsaturated dicarboxylic acids, such as dimethyl maleate, diethyl maleate, dimethyl fumarate and diethyl fumarate;

Monoolefinically unsaturated organic nitriles such as acrylonitrile, methacrylonitrile, 1,1-dicyanopropene-1, crotonitrile, oleonitrile and the like;

Monoolefinically unsaturated carboxylic acids such as acrylic acid, methacrylic acid, crotonic acid, butenoic acid, angelic acid, tiglic acid and the like;

Of these vinylidene cyanide copolymers a particularly useful copolymer which can readily be converted to filaments of excellent physical properties is the copolymer of vinylidene cyanide and vinyl acetate preferably consisting essentially of a regular structure of alternated units of the monomers, i.e., approximately 50 mol percent of each.

To improve the dyeability of the resultant fibers, the monomers making up the vinylidene cyanide copolymer may be copolymerized along with sufficient amount of an ethylenically unsaturated organic sulfonic acid to produce a copolymer containing about 0.15 to 2 mol percent of the sulfonic acid component.

Representative sulfonic acids which may be employed include styrene sulfonic acids such as ortho-, meta- or parastyrene sulfonic acid as well as commercial mixtures thereof, ortho-, meta- or para-sulfomethyl styrene, mixtures thereof, substitution products thereof such as polysulfo derivatives as well as  $\beta$ -sulfoethyl methacrylate (isethionic acid ester of methacrylic acid), sulfonic acids wherein the sulfo group is less than three atoms removed from the ethylenic unsaturation, e.g., vinylsulfonic acid, allylsulfonic acid, methallyl sulfonic acid and the like.

It is frequently desirable to employ a mixture of more than one of the foregoing vinylidene cyanide polymers in order to form fibers, e.g., a mixture of a copolymer of vinylidene cyanide and vinyl acetate and a terpolymer of vinylidene cyanide, vinyl acetate and an ethylenically unsaturated sulfonic acid or a salt thereof such as a styrene sulfonic acid or potassium styrene sulfonate. The fibers may also contain various additives in addition to the vinylidene cyanide polymer or polymers, e.g., a polymer of N,N-dimethyl acrylamide, a copolymer of N,N-dimethyl acrylamide and vinyl acetate, and so forth.

As is well known in the art, copolymers of vinylidene cyanide have particular application in the formation of fibers and generally are wet spun in order to produce such fibers.

It is an object of the present invention to provide a novel method for improving the dye receptivity of vinylidene cyanide copolymer fibers.

Another object is to provide vinylidene cyanide copolymer fibers exhibiting a superior affinity and receptivity for dyes.

Other objects and the advantages of this invention will become apparent from the discussion that appears hereinafter.

In accordance with one aspect of this invention, a spinning solution of a vinylidene cyanide copolymer is extruded through a shaped orifice into a coagulating bath which contains a minor amount of a material selected from the group consisting of polyoxyalkylene glycols and fatty acid esters of polyoxyalkylene glycols. This results in a coagulation of vinylidene cyanide copolymer fibers from the spinning solution, which fibers contain therein a minor amount of the polyoxyalkylene glycol or fatty acid ester thereof. Generally, the fiber while still in the coagulating bath, is subjected to a drawing operation, which may be followed by stretching, to provide orientation and improve the mechanical characteristics of the fiber.

The solvent employed for the vinylidene cyanide copolymer is generally a mixture of acetonitrile and water. The spinning solution solvent will usually preponderate in acetonitrile, whereas the coagulating bath will preponderate in water. For example, the spinning solution solvent mixture generally contains at least about 75 percent acetonitrile, and preferably from about 84 to 86 percent acetonitrile and correspondingly from about 16 to 14 percent water. The coagulating bath, on the other

the addition of 1% of each of the materials listed in the following table. The resulting fibers were found to take up the indicated quantities of the disperse dye, Pink BA ("Celliton Fast Pink BA-CF," General Dyestuff Co., N.Y.), after immersion for 1 hour at 97° C. of a 100 mg. portion of fiber in 600 ml. of an aqueous solution containing 300 mg. of dye. The table also includes the solubility behavior observed on mixing approximately 0.5 g. of each additive with about 2 ml. of water or acetonitrile.

| Bath Additive                                                                                  | Additive Solubility         |                          | Dye Uptake<br>(Percent Pink<br>BA in fiber) |
|------------------------------------------------------------------------------------------------|-----------------------------|--------------------------|---------------------------------------------|
|                                                                                                | In Water                    | In Acetonitrile          |                                             |
| None                                                                                           |                             |                          | 0.74                                        |
| Polyoxyalkylene Glycol, avg. molecular weight=2,900 (40% ethylene oxide, 60% propylene oxide). | Soluble room temperature    | Soluble room temperature | 1.10                                        |
| Polyoxyethylene glycol laurate                                                                 | Dispersed hot-not dissolved | do                       | 1.48                                        |
| Polyoxyethylene glycol stearate                                                                | do                          | Soluble 60° C.           | 1.52                                        |

hand, will ordinarily contain at least 55 percent water, and preferably will contain from about 62 to 80 percent water and correspondingly from about 38 to 20 percent acetonitrile.

The polyoxyalkylene materials employed in the method of our invention generally are more readily soluble in acetonitrile than in water. Such materials nevertheless have sufficient affinity for water that they will be present in significant concentration at the interface between the extruded fiber from the spinning solution and the coagulating bath, and hence will be taken up by and will be present in the resulting coagulated vinylidene cyanide copolymer fibers.

If a polyoxyalkylene glycol is employed, it is typically prepared by condensation of an alkylene oxide, e.g., ethylene oxide and/or propylene oxide, with an alkylene glycol such as ethylene glycol, propylene glycol, or the like. The polyoxyalkylene glycol should desirably have a molecular weight of from about 200 to 3,000.

In accordance with a preferred aspect of our invention, there is incorporated in the coagulating bath a fatty acid ester of a polyoxyalkylene glycol of the foregoing type.

Fatty acids which are suitable for use in preparing the fatty acid esters of polyoxyalkylene glycols may be either saturated or unsaturated. Suitable saturated fatty acids desirably may contain from about 4 to 26 carbon atoms, a more preferred range being from about 10 to 18 carbon atoms. Lauric and stearic acids are particularly suitable. Unsaturated fatty acids include those containing from about 10 to about 24 carbon atoms. A preferred unsaturated fatty acid is oleic acid.

The amount of polyoxyalkylene material present in the coagulating bath is generally from about 0.1 to 3 percent by weight, of the bath, a more preferred range being from about 0.5 to 1.5 percent.

By virtue of the foregoing method, there result vinylidene cyanide copolymer fibers which have a markedly superior dye receptivity and dye uptake. These fibers can be readily dyed with disperse dyes, as well as with acid and/or basic dyes utilizing conventional dyeing conditions and procedures.

The following example will further illustrate this invention. All parts are by weight unless otherwise stated.

#### Example

A solution was prepared consisting of 120 g. water, 680 g. acetonitrile, and 200 g. of a copolymer of vinylidene cyanide and vinyl acetate in approximately equal molar proportions. This solution, which was fluid above about 45° C., was extruded through a spinnerette containing 5 holes of 0.076 mm. diameter into a coagulation bath at 70° C., the bath being composed of 30% acetonitrile and 70% water. Fibers were withdrawn at 25 m./min. after passage through 2 feet of the bath, were wound over a pair of skewed rolls, were then remmersed in the bath for a 3 to 1 stretch between guides 1 foot apart, and finally were taken up at 75 m./min. This procedure was repeated, with the coagulation and stretch bath being modified by

20 The foregoing clearly demonstrates the improvement in dye pick-up when a polyoxyalkylene material is present in the coagulating bath as compared to a "control" where-

in the bath contains no such material.

Any departure from the above description which conforms to the present invention is intended to be included within the scope of the invention as defined by the following claims.

Having thus described our invention, what we desire to secure and claim by Letters Patent is:

1. A method of improving the dye-receptivity of vinylidene cyanide copolymer fibers, this method comprising extruding a solution of vinylidene cyanide copolymer containing more than about 45 percent vinylidene cyanide through a shaped orifice and into a coagulating bath containing a minor amount of polyoxyalkylene material selected from the group consisting of polyoxyalkylene glycols and fatty acid esters of polyoxyalkylene glycols, to thereby form and coagulate said fibers.
2. The method of claim 1 wherein said polyoxyalkylene material is a fatty acid ester of a polyoxyalkylene glycol.
3. The method of claim 2 wherein said fatty acid contains from about 4 to 26 carbon atoms.
4. The method of claim 2 wherein said fatty acid is lauric acid.
5. The method of claim 2 wherein said fatty acid is stearic acid.
6. The method of claim 2 wherein said polyoxyalkylene glycol has a molecular weight of from about 200 to 3,000.
7. The method of claim 1 wherein the amount of said polyoxyalkylene material in said coagulating bath is from about 0.1 to 3.0 percent by weight.
8. The method of claim 1 wherein said polyoxyalkylene material is a polyoxyalkylene glycol.
9. The method of claim 8 wherein said polyoxyalkylene glycol has a molecular weight of from about 200 to 3,000.
10. The method of claim 9 wherein the polyoxyalkylene units of said polyoxyalkylene glycol are selected from the group consisting of polyoxyethylene units, polyoxypropylene units, and mixtures thereof.
11. A method of improving the dye receptivity of vinylidene cyanide copolymer fibers, this method comprising extruding a solution of vinylidene cyanide copolymer containing more than about 45 percent vinylidene cyanide in a solvent mixture containing from about 100 to 80 percent acetonitrile and correspondingly from about 0 to 20 percent water, through a shaped orifice and into a coagulating bath containing from about 60 to 85 percent water, from about 40 to 15 percent acetonitrile, and from about 0.1 to 3.0 percent of a polyoxyalkylene material to thereby form and coagulate vinylidene cyanide copolymer fibers.
12. The method of claim 11 wherein said coagulated fibers are drawn down and then subjected to stretching.
13. The method of claim 11 wherein said polyoxyalkylene material is a fatty acid ester of a polyoxyalkylene glycol.
14. The method of claim 13 wherein said fatty acid contains from about 4 to 26 carbon atoms.

15. The method of claim 14 wherein said fatty acid is lauric acid.
16. The method of claim 14 wherein said fatty acid is stearic acid.
17. The method of claim 11 wherein said polyoxyalkylene material is a polyoxyalkylene glycol.
18. The method of claim 17 wherein said polyoxyalkylene glycol has a molecular weight of from about 200 to 3,000.
19. The method of claim 18 wherein the polyoxyalkylene units of said polyoxyalkylene glycol are selected from the group consisting of polyoxyethylene units, polyoxypropylene units, and mixtures thereof.

## References Cited

## UNITED STATES PATENTS

|             |         |                  |       |          |
|-------------|---------|------------------|-------|----------|
| 2,862,903   | 12/1958 | Wootton          | ----- | 260—29.6 |
| 5 3,206,420 | 9/1965  | Smart et al.     | ----- | 8—93     |
| 1,970,578   | 8/1934  | Schoeller et al. | ----- | 260—98   |

JAMES A. SEIDLECK, *Primary Examiner.*A. H. BRODMERKEL, *Examiner.*H. MINTZ, *Assistant Examiner.*